

## UNITED STATES PATENT OFFICE.

HULDREICH EGLI, OF ARBON, SWITZERLAND, ASSIGNOR TO AKTIENGESELLSCHAFT  
SEERIET, OF ARBON, SWITZERLAND, A CORPORATION OF SWITZERLAND.

## METHOD FOR IMPARTING A LINENLIKE EFFECT TO COTTON.

No Drawing.

Application filed January 2, 1926. Serial No. 79,032

Experiments for producing linen-like effects on cotton are not novel; many years ago attempts were made to obtain these effects by subjecting cotton fabric to a prolonged mercerization and to increase these effects by utilizing yarns having a higher degree of twist than such used for ordinary fabrics. The mercerizing foulards of Zittau were particularly suitable for producing these effects and they were particularly in favor for manufacturing shirtings.

Recently attempts have been made to further improve these effects. The means proposed to this end comprise in one case a cold mercerization, i. e. a mercerization at a temperature of below 0° C., and in another case an alternate cold mercerization and an acid treatment with sulfuric acid of above 50½° Bé., whereby cotton may be mercerized first and parchmentized thereafter or vice versa.

The subject matter of the present invention is a method for imparting a linen effect to cotton which is characterized by the fact that yarns or fabrics the numbering of which does not exceed count 60 are subjected to the action of sulfuric acid of from 49–50½° Bé. for a shorter or longer period depending on the count of the yarn, and are then well washed and mercerized under tension with a caustic soda solution of above 15° Bé. at a temperature of above 0° C. The invention is thus based on the observation that this method applied to coarse yarns and fabrics does not produce wool-like effects but linen-like effects.

It is a surprising result that yarns or fabrics treated with sulfuric acid of less than 50½° Bé. and subsequently treated under tension with caustic alkali of above 15° Bé. at a temperature of above 0° C. show a linen-like appearance. It is known to use sulfuric acid of less than 50½° Bé. in order to obtain effects which are softer than ordinary cotton, that is to say for effects which have a wool-like softness. The linen-like effect obtained with coarse yarns is almost the contrary of what could be expected. In order to carry out the present method ordinarily yarns of a coarseness below No. 60 English

count are utilized. Preferably the yarns or fabrics are treated with sulfuric acid of from 49–50½° Bé. at a temperature of from 0°–5° C. for a longer or shorter period, (4 minutes and more) according to the thickness of the fabrics, thereupon the products are well washed and are mercerized under tension at a temperature above 0° C. and preferably at ordinary temperatures, and are well washed. The yarns and fabric have now completely the character of linen and neither a repeated boiling nor washing will impair the strength or the gloss of the product. In order to complete the linen-like character the products are ordinarily mechanically manipulated such as by calendering same such as is customary with linen.

Having now particularly described and ascertained the nature of my said invention and in what manner the same is to be performed, I declare that what I claim is:

1. Process for producing permanent linen-like effects in cotton goods, which comprises taking for treatment cotton goods (yarns and webs) constituted of threads whose fineness does not exceed English yarn No. 75 60, and subjecting such goods to the action of sulphuric acid of from about 49° to 50½° Bé. for a period of not less than about four minutes, then washing the goods and thereafter subjecting the same while under tension to a treatment with caustic alkali of about 15° Bé. at ordinary temperatures.

2. Process for producing permanent linen-like effects in cotton goods, which comprises taking for treatment cotton goods (yarns and webs) constituted of threads whose fineness does not exceed English yarn No. 85 60, and subjecting such goods to the action of sulphuric acid of from about 49° to 50½° Bé. at a temperature of from about 0° to 5° C., then washing the goods and thereafter subjecting the same while under tension to a treatment with caustic soda of above 15° Bé. at ordinary temperatures.

3. Process for producing permanent linen-like effects in cotton goods, which comprises taking for treatment cotton goods (yarns and webs) constituted of threads whose fine-

ness does not exceed English yarn No. 60, and subjecting such goods to the action of sulphuric acid of from about  $49^{\circ}$  to  $50\frac{1}{2}^{\circ}$  Bé. at a temperature of from about  $0^{\circ}$  to  $5^{\circ}$  C. for a period of not less than about four minutes, then washing the goods and thereafter subjecting the same while under ten-

sion to a treatment with caustic alkali of above  $15^{\circ}$  Bé. at ordinary temperatures.

Dated this 16th day of December, 1925. 10

In testimony whereof I have signed my name to this specification.

HULDREICH EGLI.